

## UNITED STATES PATENT OFFICE.

JOHN L. COX, OF PHILADELPHIA, PENNSYLVANIA.

## ARMOR PLATE AND PROCESS OF MAKING SAME.

No Drawing.

Application filed January 6, 1921. Serial No. 435,535.

*To all whom it may concern:*

Be it known that I, JOHN L. COX, a citizen of the United States, residing at Philadelphia, county of Philadelphia, and State of Pennsylvania, have invented a new and useful Improvement in Armor Plate and Processes of Making Same, of which the following is a full, clear, and exact description.

10 In the manufacture of armor plate, it is a known desideratum to provide the same with a hard face and a tough back. This has heretofore been accomplished, for example, by carburizing the face of a forged plate 15 to a depth varying with the thickness of the plate, usually about eight to ten per cent of such thickness, then reforging, then heating to a high temperature to permit such rearrangement of the molecules as will produce, upon sudden cooling, a fine-grained molecular structure, suddenly cooling the plate, then reheating the plate to a lower temperature not high enough to produce hardening, then cooling slowly or suddenly, 20 then reheating the carburized face thereof to a temperature sufficient to cause hardening upon sudden cooling while heating the other side to a red heat below that necessary to produce hardening, and then suddenly 25 cooling either the whole plate or only the carburized face thereof. Part of this process is disclosed in the Ehrensberger patents No. 651,965 and No. 651,413. Other similar processes have been used.

30 35 In prior processes of the character described, the tendency has been to sacrifice the characteristics of strength and toughness of back for hardness of face. The high heat required for face-hardening is usually carried to a considerable depth below the super-carburized zone, and a layer of the general metal of the plate also heated above its hardening point and then hardened by the face-quenching to the extent that its 40 carbon content and its possible rate of cooling permit. All the metal so heated above its hardening point and quenched will show on fracture a crystalline structure. Irrespective of the thickness of the layer of back metal thus hardened, a further zone of considerable thickness will have been heated to a temperature so high as to be greatly softened and made easy of penetration.

45 50 Plates of this character may break up the older shells but the most modern projectiles are not broken up by impact upon such sur-

faces. On the contrary, the projectile cracks and spalls away the surface of the plate and penetrates the unprotected soft metal of the back, rebounding entire or completely perforating the plate, depending upon the initial energy imparted.

55 The object of my invention is to provide a carburized plate the face of which is much harder than the body or back and presents to the attack of a projectile metal highly resistant to flow, but which will neither crack nor spall; while the remainder of the plate is composed of metal with the highest available tensile strength and elastic limit 60 combined with absence of a crystalline formation which facilitates cracking and penetration. Such a back opposes continued resistance to a projectile which may have perforated the face zone, and absorbs at an unequalled rate the residual energy of the projectile.

65 Such a plate offers less resistance to superficial penetration than the plates generally in use, but more resistance to complete perforation,—which is of much greater importance; while, due to the absence of cracking or spalling, the resistance to penetration at any point is not destroyed and but little diminished by a previous exposure 70 to fire at an adjacent point.

75 The invention is particularly applicable to relatively thin armor plate—say plates of eight inches or less in thickness—although its application to even the thickest armor produces a plate which is distinctly 80 superior to a plate produced by any of the processes heretofore in general use.

85 I prefer that the plates to be treated shall have a relatively high carbon content,—say 85 from 0.34 to 0.46 per cent carbon.

90 In carburizing the plate it is distinctively preferable, although not indispensable, to carburize more deeply than heretofore. Thus, in the case of a twelve inch or thirteen 100 inch plate, I prefer to carburize to the depth of from one and one-half to two inches, while in the case of an eight inch plate I prefer to carburize to a depth of from one inch to one and one-half inches; in other words, to a depth not less than about twelve per cent 105 of the thickness of the plate.

110 I prefer that the carbon content on the face of the plate should be about 1.2 per cent—not over 1.35%—the percentage of carbon, of course, decreasing from the face toward the uncarburized body or back.

After the customary precautionary measures directed to prevent the cracking of the plate when cooled from the high temperature of carburization, the plate is cleaned and the face protected from oxidation by suitable carbonaceous covering.

The plate is then reheated to a very low forging heat, say about 1900° F., and forged down to final thickness, care being taken to work the carburized face metal as thoroughly as possible.

The whole plate is then uniformly heated to above the critical temperature for hardening, preferably to form 175° F. to 225° F. above that temperature. In the case of nickel-chrome steel of a known composition, having an average critical or  $Ac_1$  point of about 1380° F., the preferred temperature of heating would be in the neighborhood of 1600° F.

The plate is then cooled suddenly, preferably quenched by spraying. The result is a fine-grained molecular structure.

The whole plate is then uniformly reheated to somewhat above the aforesaid critical temperature, say to about 100° F. above that temperature. In the case of alloy steel, having the same critical point of 1380° F., the preferred temperature would be about 1475° F. Less preferably, the plate may be heated to a high temperature, or even to a temperature approaching or equal to that of the first heating, but in such cases, care must be exercised to limit the heating to a considerably shorter time. It is found distinctly advantageous to keep the plate at a temperature somewhat above the temperature of the critical point for a relatively long time rather than to keep it substantially above the critical point for a shorter time. The plate is again cooled suddenly, preferably quenched by spraying, as in the first heat treatment. This operation still further refines the grain.

The whole plate is then again uniformly reheated to a temperature preferably not in excess of 1225° F. and bent to shape or straightened. Any temperature used for bending which is in excess of that required by the next step is at a sacrifice of the elastic limit of the material.

After bending, the plate is uniformly reheated to a temperature above 1100° F. but so far below the critical point that after quenching no hardening will result; the plate is suddenly quenched, as by spraying.

Under certain conditions I have found it possible to give the final quench from as low as 1050° F.

If the preceding steps have been properly carried out, the plate, on fracture, will not have a granular appearance, but will have a fibrous appearance, both in the uncarburized body and through all or nearly all of the carburized face. In other words, the

fibrous appearance, instead of, as in plates treated by conventional methods, being confined to a zone at the back, leaving the entire carburized zone and a deep intermediate zone with a granular appearance, extends almost to the surface of the carburized face. The temperature of this last heating should not exceed a temperature approximately 100° below the critical  $Ac_1$  point of the steel at that stage of manufacture.

As the structure of the steel has become finer during the heat treatments described, the critical  $Ac_1$  temperature has fallen, and, for the steel chosen, at the last stage is probably not in excess of 1325° F. The quench is, preferably, at not over 1225° F., nor less than 1050° F.—the lower the better provided full fibrosity, so-called, is obtained. A temperature of about 1180° F. is usually satisfactory.

It is impossible to give more exact ranges of temperatures than those specified, because the preferred, as well as the maximum and minimum temperatures, will vary with the critical temperature of the metal, which in turn varies with the composition of the metal, as well as with the grain size.

Having now fully described my invention, what I claim and desire to protect by Letters Patent is:—

1. The process of making armor plate which comprises carburizing one face of the plate, heating the whole plate to a low forging temperature and re-forging, heating the whole plate to above the critical temperature of the metal, then suddenly cooling, heating the whole plate to at least the critical temperature, but not to the extent of the first heating, then suddenly cooling, heating the whole plate (which has thus been grain-refined) to a temperature so far below the critical temperature that, upon subsequent sudden cooling, the plate, on fracture, will present substantially throughout a fibrous appearance without substantial crystalline material, and then suddenly cooling.

2. The process of making armor plate which comprises carburizing one face of the plate, heating the whole plate to a low forging temperature and re-forging, heating the whole plate to above the critical temperature of the metal, then suddenly cooling, heating the whole plate to above the critical temperature but to a temperature lower than that of the first heating and not more than 125 degrees F. above the critical temperature, then suddenly cooling, heating the whole plate to a temperature so far below the critical temperature that, upon subsequent sudden cooling, the plate, on fracture, will present substantially throughout a fibrous appearance and then suddenly cooling.

3. The process of making armor plate

- which comprises carburizing one face of the plate, heating the whole plate to a low forging temperature and re-forging, heating the whole plate to a temperature above, but not more than 250 degrees F. above, the critical temperature, then suddenly cooling, heating the whole plate to at least the critical temperature, but not to the extent of the first heating, then suddenly cooling, heating the whole plate to a temperature so far below the critical temperature that, upon subsequent sudden cooling, the plate, on fracture, will present substantially throughout a fibrous appearance, and then suddenly cooling.
4. The process of making armor plate which comprises carburizing one face of the plate, heating the whole plate to a low forging temperature and re-forging, heating the whole plate to a temperature above the critical temperature of the metal, then suddenly cooling, heating the whole plate to at least the critical temperature but to a temperature lower than that of the first heating and not more than 75 degrees above the critical temperature, then suddenly cooling, heating the whole plate to a temperature so far below the critical temperature that, upon subsequent sudden cooling, the plate, on fracture, will present substantially throughout a fibrous appearance, and then suddenly cooling.
5. The process of making armor plate which comprises carburizing one face of the plate, heating the whole plate to a low forging temperature and re-forging, heating the whole plate to above the critical temperature of the metal, then suddenly cooling, heating the whole plate to at least the critical temperature, but not to the extent of the first heating, then suddenly cooling, heating the whole plate to a temperature not higher than 100 degrees F. below the critical temperature but sufficiently high to secure fibrosity, and then suddenly cooling.
6. The process of making armor plate which comprises carburizing one face of the plate, heating the whole plate to a low forging temperature and re-forging, heating the whole plate to a temperature above, but not more than 200 degrees F. above, the critical temperature, then suddenly cooling, heating the whole plate to at least the critical temperature but to a temperature lower than that of the first heating and not more than 75 degrees F. above the critical temperature, then suddenly cooling, heating the whole plate to a temperature not higher than 100 degrees F. below the critical temperature but sufficiently high to secure fibrosity, and then suddenly cooling.
7. The process of making armor plate, which comprises carburizing one face of the plate, purposely left somewhat thicker than its final dimension, afterward heating the whole plate to a very low forging heat and completing the forging to thickness; heating the whole plate to considerably above the critical temperature of the metal, then suddenly cooling, heating the whole plate to somewhat above the critical temperature, but not to the extent of the first heating, then suddenly cooling, heating the whole plate which has been thus grain-refined to a temperature of about 125° F., below the critical temperature of the metal, then cooling the plate, heating the whole plate to a temperature so far below the critical temperature that upon sudden cooling, the plate, on fracture, will present substantially throughout a fibrous appearance without substantial crystalline material, and then suddenly cooling.
8. The process of making armor plate which comprises carburizing one face of the plate, afterward heating the whole plate to a very low forging temperature and re-forging the plate, reheating the whole plate to above the critical temperature of the metal, then suddenly cooling, heating the whole plate to above the critical temperature but to a temperature lower than that of the second heating and not more than 125° F. above the critical temperature of the metal, then suddenly cooling; reheating the whole plate to a temperature of about 125° F. below the critical temperature of the metal, cooling the plate, reheating the whole plate to a temperature so far below the critical temperature that upon subsequent sudden cooling, the plate, on fracture, will present substantially throughout a fibrous appearance, and then suddenly cooling.
9. A heat-treated armor plate of alloyed steel, which is highly carburized from one face inward, which is substantially devoid of crystalline material, and presents, on fracture, a fibrous appearance throughout the uncarburized back, as well as the major portion of the carburized face.
10. A heat-treated non-face hardened armor plate of alloyed steel, highly carburized on one face, and of essentially uniform physical properties throughout the uncarburized portion.
11. A heat-treated armor plate of alloyed steel, carburized from one face inward to a depth in excess of eight per cent of the plate's thickness, and of substantially uniform physical properties throughout the uncarburized portion.
12. A heat-treated armor plate of alloyed steel, highly carburized from one face inward to a depth equal to a relatively small part of the thickness of the plate, substantially devoid of crystalline material and presenting on fracture, a fibrous appearance throughout the uncarburized portion, and

the major part of the carburized portion, and of substantially uniform physical properties throughout the whole of the uncarburized portion.

5 13. A heat-treated armor plate of alloyed steel, having a body whose whole minimum carbon content is not less than 0.32 per cent and which is carburized from the face in-

ward to a depth of at least twelve per cent of the thickness of the plate, the carbon content of the face not exceeding 1.4 per cent.

In testimony of which invention, I have hereunto set my hand, at Philadelphia, Pa., on this 30th day of December, 1920.

JOHN L. COX.